# EUROPEAN PATENT SPECIFICATION

(11) **EP 0 267 170 B1**
(45) Date of publication and mention of the grant of the patent: **30.01.1991**
(21) Application number: 87850297.0
(22) Date of filing: 02.10.1987
(51) Int. Cl.: B03B 7/00, C22B 1/00

(54) **Treatment of middlings**
Behandlung von Zwischengut
Traitement de barrés de triage

(30) Priority: 06.10.1986 SE 8604241
(43) Date of publication of application: 11.05.1988
(73) Proprietor: Lidström, Lars Jörgen, S-134 00 Gustavsberg (SE)
(72) Inventor: Lidström, Lars Jörgen, S-134 00 Gustavsberg (SE)
(74) Representative: Nilsson, Karl Ingvar

(56) References cited:
- DE-A- 2 417 537
- DE-B- 1 261 094
- DE-B- 2 827 924
- US-A- 2 441 584
- US-A- 3 167 502
- US-A- 3 973 736

## Description

The present invention relates to concentrating or dressing processes within the mineral processing technique, and relates more particularly to a method for use when dressing a mineral product, particularly when dressing iron ore and sulphide ore, which product has been finely divided to a particle size suitable for dressing treatment thereof in at least two stages by flotation or by magnetic separation, wherein middlings obtained during the dressing treatment are reground in order to crush individual half-grains and therewith release valuable mineral therefrom, and wherein the reground middlings are then again subjected to dressing treatment.

It is normal practice when dressing mineral products to withdraw from the process so-called middlings rich in valuable mineral, e.g. the waste or tailings deriving from a cleaner of a flotation process or from a secondary magnetic separator, and to regrind these middlings and to return the reground product to the mineral dressing process at some suitable location thereof. If, for instance, the material being dressed is obtained from a series of mills incorporating a rod mill and a downstream-connected ball mill, the middlings may be passed to the ball mill, where they are reground, but it has also been proposed to regrind the middlings in a separate tube mill. Regrinding of the middlings in ball mills and tube mills is a relatively inefficient procedure, both with regard to energy input and with regard to the increase in yield gained. There are obtained flat particle-distribution curves which exhibit an excessively large quantity of not-readily dressed fine fraction, whereas excessively large proportions of the coarse fraction of the middlings pass through the mill without being reduced sufficiently therein.

The object of the present invention is to provide a novel and useful method of procedure which will at least substantially avoid the aforesaid drawbacks encountered with known middlings- regrinding processes.

To this end it is proposed in accordance with the invention that when practicing a method of the kind recited in the introduction, the middlings are reground in a manner known per se in a mill containing an agitated grinding medium, to a particle size which is smaller than K₈₀ = 100 pm, with the aid of grinding bodies having a mean size of from 2 to 6 mm. This regrinding method, effected with the aid of comparatively small grinding bodies, results with only a relatively low energy input, in an effective attrition effect which is directed essentially to the coarse fraction of the middlings, so as to obtain a reground product which can be beneficially returned to the dressing process and which exhibits an optimum, steep particle-distribution curve.

This regrinding is effected to advantage with an energy input of at most 15 kWh/t of dry middlings, there being normally obtained herewith the desired steep particle-size distribution with desired degradation of the so-called half-grains, i.e. mineral particles which contain both valuable mineral and gangue, without at the same time forming excessive quantities of such fines which are liable to generate not-readily processed sludge or dust in the dressing equipment.

The grinding bodies used when practicing the method according to the present invention may consist of a metallic or a ceramic material, although it is normally preferred to use as grinding medium grinding bodies composed of autogenous material, e.g. a fraction selected from the material to be dressed, or a material which is rich in silicon, such as quartz or olivine. Grinding bodies which are comprised of these preferred materials are much cheaper than prefabricated metallic or ceramic grinding bodies, and result in grinding-medium residues in the reground middlings which are normally quite innocuous to the dressing process, while material which is worn away from, e.g., grinding bodies of steel, on the other hand, may cause metallic coatings to form on mineral grains, therewith rendering the concentration by flotation difficult. Problems caused by the entrainment of grinding-medium residues with the reground material, however, can normally be overcome by subjecting the reground middlings to a separate treatment to remove undesirable grinding-medium residues.

The middlings can be reground either in a dry or in a wet environment. Particularly when the invention is practiced in a dressing process which is carried out in a wet environment, such as a flotation concentration process, an advantage is gained when the middlings are also reground in a wet environment, thereby obviating the need of expensive de-watering treatment.

The invention will now be described with reference to the accompanying drawing which illustrates schematically, by way of example only, an embodiment of a plant for carrying out the method according to the invention.

References 1 and 2 in the drawing designate respectively a primary mill and a secondary mill, which in the illustrated embodiment are assumed to have the form of a rod mill 1, which receives a crushed mineral product to be dressed or concentrated, and a ball mill 2 for continued grinding of the product arriving from the rod mill 1. The product leaving the ball mill 2 is divided in a classifier 3 into a relatively fine-grained fraction, suitable for concentration, and a coarser fraction, which is returned to the ball mill for further reduction in size, in the manner indicated by the line 4. The aforesaid fine-grain fraction is passed to a concentration plant, which in the case of the illustrated embodiment is assumed to be a flotation plant that incorporates a rougher 5 and a cleaner 6. The fine-grain fraction is supplied in a substantially continual stream to the rougher 5, where the material is subjected to flotation with a suitable reagent, to form a waste or tailings containing only a low proportion of the valuable mineral or minerals concerned, these tailings being removed from the process in the manner indicated by the arrow 7. The rougher concentrate obtained in the rougher 5 is passed to the cleaner 6, in the manner indicated by the arrow 8, where there is formed, in a conventional manner, a final concentrate which contains a high proportion of valuable mineral and which is removed from the process in the manner indicated by the arrow 9, and a return product or middlings having a relatively high content of valuable mineral. These middlings are passed, in the manner indicated by the arrow 10, to a mill 11 which incorporates an agitated grinding medium, by which is meant in this patent application a mill in which a grinding effect is achieved with the aid of grinding bodies and in which the middlings that are being ground are agitated by means of an agitator that moves at a high speed. Grinding is thus accomplished as a result of pressure and shear forces which act between the grinding bodies and the middlings, these forces being generated by the agitator, which is constructed so as normally to rotate at a speed of several hundred revolutions per minute and to deliver a high power output per unit of mill volume, normally in the order of at least 10 times the power consumption per unit of mill volume of a conventional ball mill. The mill 11 operates with relatively small grinding bodies, e.g. bodies having a mean size (diameter) of 2-6 mm and, at moderate resident times with regard to the middlings being reground, will reduce the middlings to a particle size, e.g., of beneath kₐₒ = 100 pm, e.g. between k₈₀ = 20 pm and kₛₒ = 90 pm, such that so-called half-grains are crushed effectively to free particles of valuable mineral without reducing the middlings to the extreme.

The drawing shows the mill 11 provided with a rotor 12 having radially extending rotor blades 13 and stator blades 14 extending radially into the grinding chamber from the surrounding mill casing.

When the grinding bodies in the mill 11 comprise a material which is undesirable in the reground middlings, those fractions of this material which accompany the reground middlings discharged from the mill 11 may be separated out in an optional separation step 15. Grinding in the mill 11 is preferably effected in a wet environment. The reground product is returned to a suitable location in the rougher 5, for renewed flotation therein, as indicated by the arrow 16.

The material being dressed may, e.g., be a sulphide ore which is concentrated by separating therefrom gangue or oxidic iron ore which is concentrated by separating phosphorous constituents therefrom. When dressing magnetic ores, the rougher 5 and the cleaner 6 may be replaced with magnetic separators mutually connected in series.

The grinding medium may comprise grinding bodies, e.g. balls or rods, made of sintered hard metal, such as sintered tungsten carbide.

## Claims

1. A method for use when dressing a mineral product, particularly when dressing iron ore and sulphide ore, which product has been finely divided to a particle size suitable for dressing treatment thereof in at least two stages by flotation or magnetic separation, wherein middlings obtained during the dressing treatment are reground in order to crush individual half-grains and therewith release valuable mineral therefrom, and wherein the reground middlings are then again subjected to dressing treatment, characterized by regrinding the middlings in a manner known per se in a mill containing an agitated grinding medium, to a particle size which is smaller than kₛₒ = 100 pm, with the aid of grinding bodies having a mean size of from 2 to 6 mm.

2. A method according to Claim 1, characterized by regrinding said middlings at an energy input of at most 15 kWh/t of dry middlings.

3. A method according to Claim 1 or 2, characterized by using as the grinding medium grinding bodies composed of autogenous material, e.g. a fraction selected from the material to be dressed, or a material which is rich in silicon, such as quartz or olivine.

4. A method according to any of Claims 1-3, characterized by subjecting the reground middlings to a separating treatment to remove undesirable grinding-medium residues therefrom.

5. A method according to any of Claims 1-4, particularly when used with a flotation concentration process, characterized by regrinding the middlings in a wet environment.

6. A method according to any of Claims 1, 2, 4 and 5, characterized by using as the grinding medium bodies which comprise sintered hard metal, e.g. sintered tungsten carbide.

## Patentansprüche

1. Verfahren zur Anwendung bei der Aufbereitung eines Erzproduktes, insbesondere bei der Aufbereitung von Eisenund Sulfiderzen, die in eine für die Aufbereitung durch Flotation oder durch magnetische Separation in wenigstens zwei Stufen geeignete Teilchengröße fein zerkleinert sind, wobei das während der Aufbereitung erhaltene Zwischengut einem erneuten Vermahlen unterworfen wird zwecks Zerkleinerung einzelner Halbkörner und Freisetzung von nutzbaren Mineralien, und wobei das erneut vermahlene Zwischengut erneut der Aufbereitungsbehandlung unterworfen wird, dadurch gekennzeichnet, daß die erneute Vermahlung des Zwischengutes in an sich bekannter Weise in einer Mühle mit bewegten Mahlkörpern bis zum Erreichen einer Teilchengröße kleiner als k₈₀ = 100 pm unter Benutzung von Mahlkörpern mit einer mittleren Größe von 2 bis 6 mm durchgeführt wird.

2. Verfahren nach Anspruch 1, dadurch gekennzeichnet, daß die erneute Vermahlung des Zwischengutes mit einer Energiezufuhr von mindestens 15 kWh/t trockenem Zwischengut durchgeführt wird.

3. Verfahren nach Anspruch 1 oder 2, dadurch gekennzeichnet, daß als Mahlmedium Mahlkörper aus autogenem Material, wie eine Fraktion aus dem aufzubereitenden Material oder aus einem siliziumreichen Material, wie Quarz oder Olivin, verwendet werden.

4. Verfahren nach den Ansprüchen 1 bis 3, dadurch gekennzeichnet, daß das erneut vermahlene Zwischengut einem Abtrennverfahren unterworfen wird, um unerwünschte Reste des Mahlmediums zu entfernen.

5. Verfahren nach den Ansprüchen 1 bis 4, insbesondere unter Anwendung eines Flotationsanreicherungsverfahrens, dadurch gekennzeichnet, daß die erneute Vermahlung des Zwischengutes in einem nassen Medium erfolgt.

6. Verfahren nach einem der Ansprüche 1, 2, 4 und 5, dadurch gekennzeichnet, daß als Mahlmedium gesintertes Hartmetall, wie gesintertes Wolframcarbid, enthaltende Körper verwendet werden.

## Revendications

1. Un procédé utilisé dans le lavage au crible d'un produit minéral, en particulier dans le traitement de lavage au crible du minerai de fer ou des pyrites, le produit ayant été finement divisé jusqu'à une taille de particules convenable pour son traitement de lavage en au moins deux étapes par flottation ou par séparation magnétique, dans lequel les barrés de triage obtenus lors du traitement de lavage au crible sont broyés à nouveau tungstène fritté. afin d'écraser les demigrains individuels et en libérer le minéral valorisable, et dans lequel les barrés de triage rebroyés sont ensuite à nouveau sousmis à un traitement de lavage au crible, caractérisé en ce que le rebroyage des barrés de triage est réalisé d'une façon connue en elle-même, dans un moulin contenant un milieu broyeur agité, jusqu'à une taille de particules inférieure à k₈₀ = 100 pm, à l'aide de corps de broyage présentant une taille moyenne de 2 à 6 mm.

2. Un procédé selon la revendication 1, caractérisé par le rebroyage desdits barrés de triage sous un apport d'énergie d'au plus 15 kWh par tonne de matière sèche de barrés de triage.

3. Un procédé selon la revendication 1 ou 2, caractérisé en ce que l'on utilise comme milieu broyeur des corps de broyage en matériau autogène, par exemple une partie du matériau à laver, ou un matériau riche en silicium, comme le quartz ou l'olivine.

4. Un procédé selon l'une quelconque des revendications 1 à 3, caracterisé en ce que l'on fait subir aux barrés de triage rebroyés un traitement de tri qui en enlève les résidus indésirables provenant du milieu broyeur.

5. Un procédé selon l'une quelconque des revendications 1 à 4, en particulier faisant appel à un processus de concentration par flottation, caractérisé en ce que les barrés de triage sont rebroyés en environnement humide.

6. Un procédé selon l'une des revendications 1, 2, 4, et 5, caractérisé en ce que le milieu de broyage est constitué de corps comprenant un métal dur fritté, par exemple du carbure de
